

March 25, 1941.

L. SAIVES

2,235,947

PROCESS FOR THE GASEOUS CEMENTATION OF STEEL PIECES

Filed March 13, 1939

Fig-1



Fig-2



Inventor,  
L. Saives

By: Glascock Downing & Seibold  
Atts.

## UNITED STATES PATENT OFFICE

2,235,947

PROCESS FOR THE GASEOUS CEMENTATION  
OF STEEL PIECESLeon Saives, Billancourt, France, assignor to Louis  
Renault, Billancourt, FranceApplication March 13, 1939, Serial No. 261,668  
In France March 30, 1938

1 Claim. (Cl. 148—17)

The modern methods for gaseous cementation by carbon may give uniform and constant results when these are applied to furnaces in which the pieces are subject to movement, such as furnaces with rotating retort for small pieces, continuous furnaces of the propelling type, furnaces with revolving hearth, and the like, but the results are irregular in the case of cementation in stationary muffles of large size. In fact, the 5 gas inlets and outlets are also in the fixed position, and the composition of the gaseous atmosphere will gradually vary throughout the entire path of the gas, from the inlet to the discharge. The pieces which are situated outside this path 10 will be subjected to a calm atmosphere having slight whirls, and in such places the cementation is imperfect, owing to the exhaustion of the gas.

The same is true for the cementation of small pieces contained in baskets, or for the cementation 20 in the cavities of the pieces; in this case the gas is imperfectly renewed by diffusion, it becomes exhausted, and the cementation will not continue.

In the case of gaseous cementation by ammonia at about 520° C., such drawbacks have been obviated by stirring up the atmosphere by a fan which is located in the muffle and is driven by a shaft passing through the same, but for cementation by carbon, this method cannot be 25 employed, owing to the very high temperature, which is between 800° and 1000° according to the case (usually about 930°).

The present invention consists in obtaining, by a static method and without any heated mechanism, the homogeneous nature of the gaseous composition throughout the whole of the cementation muffle.

For this purpose, I produce sudden periodic variations of pressure having a great value. For 40 instance, by any suitable method which can be readily conceived, I suddenly send into the cementation muffle a volume of gas comparable with the volume of the muffle. This will cause a sudden increase of pressure, but owing to the gas 45 discharge conduit and to the inevitable leakage at the charging door (even though this is as tight as possible), the pressure will gradually fall to a value near atmospheric pressure. At this time, 50 i. e., in a few minutes, another sudden supply of gas will increase the pressure.

The frequency of this pulsatory action is sufficiently low in order that at each instant the equilibrium of pressure shall be practically attained 55 at all points of the muffle. The admission

of gas is sufficiently abrupt in order that the rise of pressure shall be as great as desired.

The volume of gas supplied at each pulsation, the time between any two pulsations, and the rapidity of the injection, are regulated according to the volume of the muffle, the leakage at the charging door (or at the evacuation conduit), and the supply of gas required for a uniform and homogeneous cementation. 5

For operating the process, the subject-matter 10 of the invention, use may be made of various devices adapted to provide a periodic supply of a large quantity of gas.

As examples which are not of a limitative nature, the following description relates to two such 15 devices, with reference to the two figures of the accompanying drawing, in which

Fig. 1 is a diagrammatic view of one form of device for practicing the process of the invention, certain of the parts being shown in full lines 20 and certain other parts shown in section, and

Fig. 2 is a similar view of another form of device for practicing the invention.

The device which is shown diagrammatically in Fig. 1 comprises a supercompressor 1 which receives—through the pipe 2—the gas supplied by the preparatory apparatus and delivers this gas into a recipient 3, whose periodic discharge into the cementation muffle 4 is assured by a gate-valve 5 which is controlled by the maximum pressure prevailing in the recipient 3, or by a clockwork device. At each discharge, the pressure rises rapidly in the interior of the muffle, and then falls more slowly until the next discharge, owing to the exit of the exhausted gas 35 through the evacuation conduit 6 or to leakage which may occur in spite of the tight door 7. 30

In the device shown diagrammatically in Fig. 2, the recipient 3 is replaced by a compressible rubber bag 8 which is supplied through a gate-valve 9 and discharges through a gate-valve 10. The discharge from the bag may be obtained by compressing the said bag by means of a fluid (compressed air or water under pressure) which is sent around the bag into a recipient containing this latter. The said fluid is delivered into the recipient through a gate-valve 12, and it is discharged through a gate-valve 13. The valves 9 and 10 on the one hand, and 12 and 13 on the other hand, are automatically controlled in such 45 manner (for instance) that the valves 9 and 13 will be opened and the valves 10 and 12 will be closed during the filling of the bag, and that the valves 9 and 13 will be closed and the valves 10 and 12 opened during the emptying of the bag. 50 55

The valves 9, 10 and 12, 13 may be controlled by electric means or by clockwork; and they may be combined together or assembled in a single apparatus.

5

I claim:

In a process for the cementation of steel articles in a stationary muffle, the step which consists in periodically supplying fresh cementation

gas under high pressure intermittently to the muffle, whereby the pressure in the muffle will rise abruptly and will then gradually fall to its initial value whereby fresh cementation gas comes in contact with all parts of the surface of the steel articles.

LEON SAIVES.